

# UNITED STATES PATENT OFFICE.

JOHN W. GEBHARD, OF MUNCIE, INDIANA, ASSIGNOR TO ARMOR STEEL & FOUNDRY COMPANY, OF CHICAGO, ILLINOIS, A CORPORATION OF ARIZONA TERRITORY.

## PROCESS FOR HARDENING STEEL CASTINGS.

1,015,554.

Specification of Letters Patent. Patented Jan. 23, 1912.

No Drawing.

Application filed May 15, 1909. Serial No. 496,125.

*To all whom it may concern:*

Be it known that I, JOHN W. GEBHARD, citizen of the United States, residing at Muncie, in the county of Delaware and State 5 of Indiana, have invented certain new and useful Improvements in Processes for Hardening Steel Castings, of which the following is a specification.

This invention relates to improvements in 10 processes for producing a "chill", or hardened face on soft steel castings, and the improvements which form the subject-matter of this application constitute a modification of the process described in a pending application for patent filed by me Sept. 21, 1906, 15 under Serial No. 335,535. In the working of the process covered by said application for patent, it has been found that in making castings of large size, the molten steel 20 retains its heat sufficiently long to effect a perfect fusing of the high-carbon coating composition and the common steel base or body without the aid of either silica or aluminum, hence in producing such castings 25 these elements may be omitted. It has also been found that in producing light castings, valuable results are attained by mixing with the manganese, which is the basis of the coating compound, other elements such as 30 vanadium, ferro-chrome and tungsten either separately or collectively, hence I desire to protect by Letters Patent, the use of these and other elements of a similar nature when combined with manganese or other high 35 carbon metallic products, and a suitable oil or liquid binder which will have a beneficial effect when subjected to the action of the molten metal.

The specific process herein referred to 40 differs from that described in the pending application above mentioned only in the composition applied to the face of the mold, hence I will not repeat in detail the description of the various steps of said process.

45 The compound or composition consists of finely ground manganese or similar element, containing a relatively large per cent. of carbon, and finely ground ferro-chrome in the proportions of twenty pounds of the manganese to eight ounces of ferro-chrome. 50 These elements are thoroughly mixed together, and when it is desired to apply the mixture to the portions of the mold where the chilled surface is to be produced in the

casting, linseed oil is mixed with the 55 powdered elements in sufficient quantities to form a thin paste which is then applied to the face of the mold, forming a coating which covers the indicated portions of the mold to the desired depth. It has been 60 found that the depth of the "chill" or hardened skin on the casting when produced from a mold thus treated is approximately 65 double the thickness of the coating, so that if a skin one-eighth of an inch thick is desired on the casting the paste will be applied to a depth of one-sixteenth of an inch.

While I have found that linseed oil makes the most effective binder for the comminuted metals, I have also used a commercial product known as "glutene" with fairly good results. I understand that this product is a kind of glue made from fish. Hence I do not wish to be limited to a vegetable oil as a 70 binder for the metallic elements named, as 75 an animal oil or a glutinous compound or substance may be used in lieu of the oil mentioned.

It should be understood that the oil or other substance used as a binder in this process, has an additional function of generating a high degree of heat when subjected to the molten metal, which facilitates the fusing of the coating compound with the body of the steel mass, and as it gasifies quickly, it 80 also aids in carrying off the other gases produced from the molten steel, thus tending to 85 eliminate blisters from the finished product. The quantity of oil used with an admixture of twenty pounds of manganese and eight 90 ounces of ferro-chrome, is about five ounces.

In producing a casting in a mold coated with the above compound, it has been found that the elements of the compound are fused by the molten steel and uniting with the 95 latter produce a hard and dense facing upon the casting at the points corresponding to the portions of the mold so treated. The texture strength and hardness of this facing depend upon the high carbon properties of 100 the substances used. The fusing is facilitated by the oil which not only forms a binder for the comminuted minerals present, but aids combustion.

Having thus described my invention what 105 I claim is:—

1. In the art of making steel castings, a paste composed of a finely ground manga-

nese, finely ground chrome and a liquid binder adapted to be applied to the face of the mold from which the casting is produced.

2. In the art of making steel castings, a  
5 paste composed of finely ground manganese,  
finely ground chrome and an oily binder  
adapted to be applied to the face of the mold  
from which the casting is produced.

3. In the art of making steel castings, a  
10 paste composed of finely ground manganese,  
and finely ground chrome and a vegetable  
oil binder.

4. In the art of making steel castings, a  
paste composed of finely ground manganese,  
finely ground chrome and an oil binder in <sup>15</sup>  
substantially the following proportions:  
Manganese 20 pounds; chrome 8 ounces; oil  
5 ounces.

In testimony whereof I affix my signature  
in the presence of two witnesses.

JOHN W. GEBHARD.

Witnesses:

H. DE LOS HIGMAN,  
F. BENJAMIN.

---

Copies of this patent may be obtained for five cents each, by addressing the "Commissioner of Patents,  
Washington, D. C."

---